

Jan. 5, 1971

KIYOSHI OTAKA

3,552,032

METHOD AND EQUIPMENT FOR RELAX SETTING

Filed May 14, 1968

5 Sheets-Sheet 1



Jan. 5, 1971

KIYOSHI OTAKA

3,552,032

METHOD AND EQUIPMENT FOR RELAX SETTING

Filed May 14, 1968

5 Sheets-Sheet 2



Fig. 5



Jan. 5, 1971

KIYOSHI OTAKA

3,552,032

## METHOD AND EQUIPMENT FOR RELAX SETTING

Filed May 14, 1968

5 Sheets-Sheet 3



Jan. 5, 1971

KIYOSHI OTAKA

3,552,032

METHOD AND EQUIPMENT FOR RELAX SETTING

Filed May 14, 1968

5 Sheets-Sheet 4

Fig. 4



Jan. 5, 1971

KIYOSHI OTAKA

3,552,032

## METHOD AND EQUIPMENT FOR RELAX SETTING

Filed May 14, 1968

5 Sheets-Sheet 5

Fig. 6



## 1

3,552,032

## METHOD AND EQUIPMENT FOR RELAX SETTING

Kiyoshi Otaka, 187 Gyogazuka Ikenoue,

Itami, Hyogo Prefecture, Japan

Filed May 14, 1968, Ser. No. 729,070

Claims priority, application Japan, May 18, 1967,

42/31,609

Int. Cl. F26b 3/00

U.S. Cl. 34—9

5 Claims

## ABSTRACT OF THE DISCLOSURE

A method and equipment for relax setting and creping, wherein fabric is treated within a rotating drum which is heated by dry hot wind or steam, and the fabric thus treated is free from such defects as creasing, unlevel creping, etc., that are usually experienced with the treatment by the washer which uses hot water.

This invention relates to an improvement in the method for relax setting and has for an object to provide a novel method of relax setting and a device of a new construction necessary for carrying out such method. The recent tendency is that tricot, raschel and other fabrics made of synthetic hard-twisted yarn or textured yarn are increasing rapidly. These fabrics are generally given a beating treatment in hot water so that they may be relaxed or in some cases creped, thereby displaying their own elasticity, solid feeling, bulkiness, soft feeling, etc. These creping processes are usually done by using the washer but the following disadvantages are experienced with the treatment by the washer, i.e., (1) inefficiency due to the batch system, (2) difficulty of controlling the processing conditions and (3) a high incidence of troubles, such as creasing, wrinkling, uneven creping, etc.

The present invention has for an object to provide a novel method for relax setting which is free from such disadvantages as mentioned above and a relax setting apparatus of a new construction necessary for carrying out such a novel method. According to the present invention, a plate having many perforations is shaped into a cylindrical form, in which a drum having several ledges protruding axially is installed. By treating fabrics in this drum which is being heated and turned, a complete relaxing effect and a creping effect can be obtained efficiently and under perfect control, without such troubles as creasing, wrinkling, unlevel creping, etc., as usually experienced with the washer or other relaxing machines.

The nature and further advantages of the present invention will be known more clearly from the following descriptions made with reference to the accompanying drawings, in which:

FIG. 1 is a side view in vertical section of the basic construction of the invention,

FIG. 2 is a front view, in vertical section, of FIG. 1,

FIG. 3 is a side view, in vertical section, of an embodiment which is different from those shown in FIGS. 1 and 2,

FIG. 4 is a front view of a power transmission apparatus in FIG. 3,

FIG. 5 is a side view of FIG. 4, and

FIG. 6 shows a device to be used for the embodiment No. 3 in the description.

Numerals 1 denotes a cylindrical body lined with a heat-

## 2

insulating layer 4. Arranged in this body are stays 1a, 1a . . . so as to make the body in good shape. Numeral 2 denotes a drum supported by a plurality of receiving roll 5b and pressing roll 5a within the body. This drum has many perforations, each of about 8 mm. in diameter, 2a, 2a . . . all over its surface and also has therein six to eight stainless steel ledges (10-15 cm. in height) provided protruding at regular intervals in parallel with the axial direction or with a proper gradient. Steam or hot air is supplied into this drum 2 or, in some cases, it may be so designed as to supply heat-source, such as hot air, steam, etc., into the gap between the outer surface of the drum 2 and the body 1. The body 1 is provided with a peep-window for inspecting the inside. This peep-window has a cover 6a so that the inside can be inspected as the occasion demands. Connected with the body is an exhaust cylinder 7, which carries dampers 9 therein. Connected with the exhaust cylinder 7 and outside the dampers is an exhaust fan 8, which, together with dampers, regulates exhausting. As indicated by the solid line in FIG. 1, introduced in the gap between the drum 2 and the body 1 is a tube 10 which supplies steam or hot air into the machine. This tube carries many nozzles 11, 11 . . . within the machine and through the medium of these nozzles the drum 2 is heated. As indicated by a chain line in FIG. 1, this tube 10 can be introduced into the drum 2 to discharge steam through its nozzles into the drum. Provided at the front portion of the drum 2 is a hopper in which fabric L is fed and provided at the end portion of the machine is an outlet 13 from which treated fabric is sent out.

FIGS. 3-5 show respectively a different embodiment from that shown by FIGS. 1 and 2. The different points in construction from FIGS. 1 and 2 are that the duct 15 is provided at the front portion and at the rear portion of the drum 2, the supplying apparatus which supplies hot air, steam, etc., to the duct is installed and the fabric feeding device 12a of different construction is added. The drum which is supported by receiving rolls 5b, 5b . . . and pressing rolls 5a, 5a . . . is driven by an electric motor M through the intermediate chain wheels Ma and Mb, cogwheel 16 and cogwheel 17 secured to the drum 2.

While heating the inside of the drum 2 by dry hot air or saturated vapor, rotate the inside of the drum at 40-60 r.p.m. in the right and the reverse directions alternately, for about 10 seconds in each direction. When material fabric is put in this drum 2, the fabric is beaten incessantly against the inside wall of the drum due to the movement of the ledges caused by the revolution of the drum and the gravity of the fabric itself. Such mechanical movement, coupled with the heating treatment by dry hot air or steam heating, imparts satisfactory relaxing effect and heat setting effect to the fabric. As compared with the washer or the like, since the present invention uses no hot water, the fabric under treatment has no added weight to the weight of itself and accordingly beating force is not so strong as in the case of the washer. Moreover, since the r.p.m. of the drum is relatively high, the fabric under treatment is uniformly rubbed and beaten, with the result that it is free from creasing, wrinkling, and unlevel creping.

If the drum is made about 10 meters in length and the axis of rotation of the drum is slanted, or, as indicated by the drawing, if the component force of centrifugal force is utilized by making the diameter of the outlet larger than that of the inlet of the drum, it is possible

to make the fabric under treatment move slowly in the drum and accordingly it is made possible to carry out relax setting continually. In this case by making the fabric stay (idle) at the outlet and at the inlet of the drum, it is possible to check the twisting of the fabric due to the revolution within the drum extending to that part of the fabric before and after treatment.

#### EMBODIMENT NO. 1

Prepare a cylindrical drum 2 made of 1 mm. thick stainless steel, with many perforations of 8 mm. in diameter (perforations rate—50%), an inlet of 90 cm. in diameter, an outlet of 100 cm. in diameter, and 1,000 cm. in length. Provided in the cylindrical drum are eight ledges 3 of stainless steel at regular intervals, each 13 cm. in height. The axis of rotation of the drum is positioned horizontally and the above-mentioned ledges are arranged in parallel with or across the axial direction. The drum is kept turning at the speed of 42 r.p.m. in the right and the reverse directions alternately, for 10 seconds in each direction, and the inside of the drum is kept at the temperature of 100° C. If tricot half fabric knitted at 28 gauges, c.p.i. 44 and w.p.i. 28, with polyester filament 20-denier as back and polyester wooly textured yarn 75-denier as front, is treated continually in the drum, the fabric will reach the outlet automatically in about 20 minutes. The fabric thus treated, as compared with that before treating, has shrunk about 40% in a width direction and about 25% in a lengthwise direction, and has satisfactory bulkiness, elasticity, solid feeling, soft feeling, etc. as tricot fabric woven with wooly textured yarn.

The fabric treated in the above way is free from creasing, wrinkling and unlevel creping. Moreover, at the subsequent processes, such as scouring, dyeing and finishing, it is almost free from the reduction of bulkiness, stretching due to tension and creasing of rope-shape. In other words, the above method will produce a perfect relax setting effect.

#### EMBODIMENT NO. 2

While turning the same machine as used in embodiment No. 1 at 48 r.p.m. in the right and the reverse directions alternately, for 10 seconds in each direction, keep the inside of the drum at temperature of 100° C. by saturating superheated steam, paying attention to drain.

If the fabric of amunzen construction with polyester filament (75-denier, twist number 1,600 T/M) used as warp and polyester wooly textured yarn 75-denier and polyester filament 75-denier (twist number 300 T/M) used as fillings—192 warps/3.79 cm. and 194 fillings/3.79 cm.—is put in the inlet of the drum under the above-mentioned condition, the fabric will reach the outlet in 20 minutes. The fabric thus treated, in comparison with the fabric before treating, has shrunk 50% in a width direction and 25% in a lengthwise direction, with the result that ideal creping effect can be obtained.

Besides the above-mentioned embodiment, circular-knitted fabric, weft-knitted fabric (using textured yarn), elastic fabric or the like can be given similar relaxing and creping by this method. In cases where the fabric for treatment has been woven using hard sizing agent, it must be desized before treating. In this case, if the drum is heated by supplying dry hot air in larger quantities to treat the desized fabric in the drum, as well as for drying, the desired relaxing effect can well be obtained.

#### EMBODIMENT NO. 3

In this embodiment, a device shown in FIG. 6 is used. This device is a combination of relax setters A and B shown in FIGS. 1 and 2 or in FIGS. 3, 4 and 5, each comprising a single drum. A washing apparatus C is provided in front of the front relax setter A and a scutcher 18 which puts treated fabric in order is provided at the back of the rear relax setter B. The fabric L which was cleansed in the washing apparatus C is given washing

and relaxing by hot water at A supplied via pipe P from a suitable source S, FIG. 6. Then, it is given finishing relaxing by steam at B and is finally taken out by the scutcher 18 and is folded.

Under this invention, it is possible to raise the relaxing effect by using hot water together as indicated by embodiment No. 3 (for example, hot water is added to the W position in FIG. 1).

From the foregoing description, it will be seen that according to the present invention, excellent relaxing and other effects as indicated by the above-mentioned embodiments can be obtained.

Having thus described the nature of the present invention, what I claim is:

1. A method of relax setting of fabrics comprising introducing a length of fabric into one end of a rotary treatment zone, supplying a heating medium selected from the group consisting of hot air and steam to the interior of said zone, alternately rotating such zone in opposite directions, beating such fabric length within such zone in the presence of such heating medium and removing such length of fabric from the opposite end of such zone.

2. A method of relax setting of fabrics as claimed in claim 1 and further including subjecting such fabric length to a pre-treatment just prior to introducing the same into said rotary treatment zone by feeding the same into one end of another and longitudinally aligned rotary treatment zone, supplying hot water to the interior of such another treatment zone, alternately rotating such another rotary treatment zone, beating that portion of the fabric length within such another rotary treatment zone while in the presence of such hot water, withdrawing such fabric length from the other end of such another treatment zone and introducing the same into said first mentioned rotary treatment zone.

3. A method of relax setting of fabrics in a rotary perforated drum having an inlet at one end and an outlet at the other end and also having internal, circumferentially spaced, inwardly projecting vanes extending substantially throughout the length of said drum, comprising introducing one end of a fabric length into the inlet end of such drum, removing such fabric length from the outlet of such drum, supplying a heating medium selected from the group consisting of hot air and steam to the interior of such drum, and alternately rotating such drum in opposite directions so as to subject the fabric while in the interior of such drum to the action of such heating medium and to beat the fabric against the interior of such drum due to the movement of the vanes caused by the rotation of the drum and the force of gravity acting on the fabric while it is inside the drum.

4. Apparatus for relax setting of fabrics comprising a cylindrical heat-insulating casing means, a drum within said casing means, said drum including side wall means and opposite end wall means, means within said casing means and operably related with said side wall means for rotatably supporting said drum, said side wall means having perforations therein, means defining a fabric inlet operably associated with one end wall means, means defining a fabric outlet operably associated with the opposite end wall means, a plurality of circumferentially spaced, inwardly projecting vanes mounted on the inner surface of said side wall means and extending substantially throughout the length of said side wall means, means operatively associated with said fabric inlet for introducing a length of fabric into the interior of said drum, said length of fabric being removed from the fabric outlet, means for supplying a flowable heating medium to the interior of said drum, heating medium outlet means operably associated with said casing means, and means for rotating said drum.

5. Apparatus for the relax setting of fabrics as claimed in claim 4 and a second casing means arranged adjacent to and in alignment with said first casing means, a second drum within said second casing means, means within said

second casing means for rotatably supporting said second drum, said second drum including side and opposite end wall means, a fabric inlet on one end wall means, a fabric outlet on the other end wall means, said last mentioned fabric outlet being aligned with the fabric inlet of said first mentioned drum, a plurality of circumferentially spaced inwardly projecting vanes arranged on the inner surface of said side wall means of said second drum and extending substantially throughout the length of said side wall means of said second drum, means operatively associated with the fabric inlet of said second drum for feeding a fabric length into the interior of said second drum, said fabric length passing through the fabric outlet of said second drum and into the fabric inlet of said first drum,

and means for supplying hot water to the interior of said second drum.

**References Cited****UNITED STATES PATENTS**

- |   |           |         |               |       |        |
|---|-----------|---------|---------------|-------|--------|
| 5 | 2,452,134 | 10/1948 | Lowe          | ----- | 34—127 |
|   | 2,735,226 | 2/1956  | Franks et al. | ----- | 34—129 |
|   | 2,898,099 | 8/1959  | De Coriolis   | ----- | 263—34 |

JOHN J. CAMBY, Primary Examiner

U.S. CL. X.R.

34—127

10